

# UNITED STATES PATENT OFFICE.

ROBERT T. STAPLES, OF NEW YORK, N. Y., ASSIGNOR TO WESTERN ELECTRIC COMPANY, INCORPORATED, OF NEW YORK, N. Y., A CORPORATION OF NEW YORK.

## CONDENSER AND THE METHOD OF MAKING SAME

1,425,912.

Specification of Letters Patent. Patented Aug. 15, 1922.

No Drawing.

Application filed August 17, 1920. Serial No. 404,254.

To all whom it may concern:

Be it known that I, ROBERT T. STAPLES, a citizen of the United States, residing at New York, in the county of New York and State of New York, have invented certain new and useful Improvements in Condensers and the Methods of Making Same, of which the following is a full, clear, concise, and exact description.

10 This invention relates to condensers and the method of making the same, the object being to provide an improved method for treating condensers so that their electrical constants are quickly brought to 15 a permanent value and to prevent further change in such constants as a result of normal temperature changes.

20 In various telephone and telegraph circuits there is a demand for a condenser, the capacity of which is held to very close limits and cannot change materially without effecting the operation of the circuit. For such purposes it is a common practice to 25 employ a condenser of the general type disclosed in Patent No. 1,200,063 of October 3, 1916, to Wheeler and Sultzzer. This condenser consists of alternate sheets of conducting and insulating materials held between a pair of heavy plates, the unit preferably being impregnated in a paraffine 30 compound. In condensers used heretofore, considerable difficulty has been experienced due to the change in capacity and it has been a customary practice to place such condensers on a shelf for a period of at least 35 nine months in order to allow their electrical characteristics to become constant.

40 In accordance with the present invention, the condenser units are placed in an oven at a temperature slightly below the melting point of the impregnating compound, and left at this temperature for a time sufficient to allow the units to become uniformly heated throughout. In the case 45 of condensers which are impregnated with a paraffine wax, the solidifying temperature of which is approximately 120° F., it has been found satisfactory to maintain the oven at a temperature of approximately 110° F. 50 and to keep the condenser units at such temperature for a period of approximately four hours.

Although it is the practice in connection with paper condensers which are sealed in a container to permanize the condensers by heating them at a temperature in excess of the melting point of the impregnating compound as disclosed, for example, in Pruessman Patent 1,275,468 of August 13, 1918, such a process is not satisfactory in connection with mica insulated condensers which are not placed in a container. With such units, if the impregnating wax is allowed to reach the melting point, a certain amount of this wax flows out, thus changing the capacity of the unit and also when the impregnating wax changes from a solid to a liquid state or vice versa, the sudden change in volume causes erratic results. By employing a temperature at which the impregnating wax only becomes plastic, all internal stresses within the unit are allowed to dissipate and the unit quickly attains its permanent capacity value.

What is claimed is:

1. The method of treating a condenser comprising an impregnated unit which consists in heating said impregnated unit to a temperature slightly below the melting point of the impregnating compound and maintaining the unit at such temperature for a period of time sufficient to allow the unit to assume its natural shape.

2. The method of treating a condenser comprising a unit impregnated with a paraffine compound having a solidifying temperature of approximately 120° F., which consists in heating the impregnated unit to a temperature of approximately 110° F. and maintaining said unit at this temperature for a period of not less than three hours.

3. The method of treating a condenser comprising an impregnated unit which consists in heating said impregnated unit to a temperature at which the impregnating compound becomes plastic, but does not become fluid and maintaining the unit at such temperature for a period of time sufficient to allow the stresses therein to become dissipated.

In witness whereof, I hereunto subscribe my name this 11 day of Aug. A. D. 1920.

ROBERT T. STAPLES.